

## UNITED STATES PATENT OFFICE

2,615,825

METHOD EMPLOYING AMINES FOR  
CLEANING TYPE MATRIXES

William Heinecke, New York, N. Y.

No Drawing. Application October 24, 1946,  
Serial No. 705,481

14 Claims. (Cl. 134—2)

1

This invention relates to the cleaning of metal such as brass and more particularly to the cleaning of matrixes used in the casting of integral lines of type.

In the founding of integral lines of type, or in the Linotype process, matrixes for each letter are arranged into a line mold for casting a slug corresponding to a line of separate type. After the casting of a slug, the individual matrixes are automatically sorted and returned to their respective prearranged locations where they may again, by manually controlled automatic machinery, be arranged to form another mold for another slug.

These matrixes are in fact precision dies. For instance the side walls on some dies for some characters are about .001 inch thick and of height equal to the relief of the cast type. In the founding it is of utmost importance that outer faces of these side walls be flat against outer faces of those of an adjacent matrix, otherwise a vertical line between letters will be printed from the cast slug.

In use, the matrixes are subjected to extreme pressures to prevent any leakage of molten metal between the several aligned matrixes. Moreover it is necessary to insert wedges called space bands between the characters at word intervals to justify the line of type. These space bands are coated with graphite for lubrication as they must be forced in between the matrixes. In course of time, the matrixes have a coating of graphite built up upon them and the delicate side walls are caved in due to the pressures involved. Also deposits other than graphite occur on the matrixes and are the result of various origins. Such deposits may be lead sulfide, ordinary corrosion due to atmospheric action and particles of dust which are ever present. Another objection to the presence of these deposits or grime is that the character stamped on the edge face of the matrix becomes indistinct so that the operator cannot read the line in the process of composition so that errors frequently occur.

Numerous means for cleaning the matrixes have been employed and are still in use. Brass wire brushes are used extensively on a group of matrixes but only on their "ears" and "toes" or other durable parts of the matrix. The side faces are then rubbed manually on a soft pine board each matrix being handled one at a time. Since a set of matrixes for each machine may number about 1500 the process is tedious and costly and furthermore the character die is never cleaned at all. One manufacturer recommends the use of

2

a rubber eraser, but not on the die. Each of these processes is liable to form grime or burrs which are likely to cave the side walls, as well as prevent the falling of the matrix from the magazine.

5 Thus, by these processes no real cleaning is effected except to the extent to make the character stamp more easily read.

Many liquid cleaners have been employed for the removal of the grime from matrixes but none has been altogether satisfactory. Chromic acid has probably been more generally used than any other liquid but this material is highly corrosive so that special materials must be used for the cleaning tanks. Furthermore, and of greater importance, chromic acid is corrosive to the matrixes, usually of brass, so that their dies lose their distinction. Distinction is lost by the corrosion of side walls, pitting of the die which causes specks on the printing, and deepening of the die which raises the type of some letters so that an uneven print job is the result. This corrosion occurs even though the matrix is washed subsequent to the cleaning, and of course the use of chromic acid is dangerous to the operators. In use the chromic acid gradually becomes exhausted and must be replenished from time to time, always carefully to minimize the corrosion. The chromic acid process requires much time for each matrix must be laid aside to allow a complete evaporation of the wash water.

30 I have found that free alkyl amines and alkanol amines are effective at room temperature for the rapid elimination of the grime from the matrix, and yet the brass of the matrix is not attacked. Ordinarily the amines employed are much more volatile than water and certainly more volatile than chromic acid or sulfuric acid which is usually associated with the chromic acid. Hence matrixes may be immersed in the amine and then dried with only an absorber or an air blast. However I prefer to wash the adhering amine from the matrix with a volatile chlorinated hydrocarbon such as carbon tetrachloride or tetrachloroethylene since these two are non-inflammable. Preferably the chlorinated hydrocarbon should contain a small amount of acid material such as hydrochloric acid or sodium bisulfate, the latter preferably since it is heavy enough to remain quiescent at the bottom of the liquid and is insoluble.

45 Finally the amine, or neutralizing wash liquid if the latter is used, is removed from the matrixes by means of an air blast or the matrixes may be tumbled or exposed in an absorber chamber. For example, the matrixes may be passed over acti-

vated carbon for the removal of the amine or the chlorinated hydrocarbon.

To carry out my process I agitate the matrixes in the amine either with or without means such as brushes to disengage coarse grains. The amine may be an alkyl amine or an amino alcohol. Preferably the amine should be a non-toxic and non-inflammable liquid. However, if the amine is inflammable, as for instance diethyl amine, a little water may be added to the amine to lower the vapor pressure. It has been found that many of the amines almost instantly separate the grime from the matrixes. I prefer to use amines such as mono ethanol amine or ethylenediamine since neither of these is extremely volatile but yet both are very efficient. Other amines which may be used include diethyl amine, triethyl amine, methyl amine, dibutyl amine, tributyl amine, diamyl amine, triamyl amine, diethylamino ethanol, ethyl ethanol amine, ethyldiamino amine, ethyl diethanol amine, butyl ethanol amine, butyldiethanol amine, dibutyl amino ethanol, diethyl amino ethanol, and hexylamine.

Generally I prefer that the carbon chains of the amine contain less than seven carbon atoms and when secondary or tertiary amines are used I prefer the number to be less than six.

After the matrixes have been cleaned they are preferably dipped in a solvent wash to remove any adhering amine. While I prefer tetrachloroethylene as the solvent wash because of its low toxicity and non-inflammability obviously other liquid washes which will remove the amine may be used. If a hot air blast is used as the final absorber or drier, water alone may be used for the wash. However, acid material should preferably not be used in the water as it will adhere to the matrix and cause corrosion. On the other hand when a chlorinated hydrocarbon is used as the liquid, sodium bisulfate or other acid material not soluble in the liquid merely absorbs the amine from the liquid by constant contact therewith. After a long period of use the sulfate salt may be removed from the liquid by filtration and a fresh supply of bisulfate added.

The chlorinated hydrocarbon wash has the advantage that no frequent changes of wash water are required which would either be inconvenient if supplied manually or require pipe connections if supplied more or less automatically.

The wash liquid need not be pure carbon tetrachloride or the like for I may employ a mixture of ethyl or isopropyl alcohol and carbon tetrachloride which will not be inflammable. Similarly trichloroethylene may be used with the alcohols. In fact the only major requirements of the wash liquid are that it be a solvent for the amine, readily evaporated and not corrosive to the matrix. However non-inflammability enables the use of a simple tank.

The adhering wash liquid may be removed from the matrix by well known means as by an air blast which will not contain abrasive material to injure the definition of the code slot or the character molds.

The reason for the activity of amines in the cleaning of the matrixes is not understood. Some amines have been known to be good degreasing agents and yet degreasing agents have been almost universally rejected for cleaning matrixes in favor of the chromic acid treatment. Chromic acid is apparently effective by virtue of its strong oxidizing or corrosive properties and yet ethylene diamine used as a corrosion inhibitor in anti-freeze solutions, is very effective

for loosing the graphite and lead sulfide from the matrix. The problem has evidently been solved by applicant in a way different from the mere dissolving of grease. Perhaps the initial action of the amine dissolves grease and then complex copper or zinc ions form a protective film on the surface of the matrix and this film may work itself under particles of lead sulfide or graphite causing the latter to slough off.

The choice of a particular amine will depend on the requirements of each individual situation as determined by the requirements for speed, fume confinement, ventilation, exposure to fire and the like. Thus where speed is especially required I prefer to use amines having less than three carbon atoms to each aliphatic group, such as ethanalamine, ethylenediamine, ethylethanol amine, ethyldiethanolamine, diethyl amine. Obviously various mixtures of these amines, or others mentioned herein, may be blended to form liquids having different degrees of viscosity or volatility. For instance, methyl amine alone would require special care because of its low boiling point, however if it is mixed with viscous ethanalamine the mixture is safe and will not adhere to the matrix to the same degree as will ethanalamine.

The invention claimed is:

1. A method for cleaning grime containing lead sulfide and graphite from brass matrixes for integral line type and comprising washing the matrixes at room temperature in a free amine which is liquid at room temperature.
2. A method for removing lead sulfide and graphite from brass matrixes for integral line type and comprising washing the matrixes at room temperature in ethylenediamine, the latter having the double function of a cleaner and corrosion inhibitor.
3. A method for ridding brass matrixes of grime containing lead sulfide and graphite which method comprises washing the matrixes at room temperature in an aliphatic amine which is liquid at room temperature.
4. A method as in claim 3 said amine being a primary amine and any carbon chain thereof having less than seven carbon atoms.
5. A method as in claim 3 said amine having more than one carbon chain attached to the nitrogen and any chain having less than six carbon atoms in the chain.
6. A method for removing grime containing lead sulfide and graphite from brass matrixes for integral line type, said method comprising washing the matrixes at room temperature in an alkanol amine which is liquid at room temperature, the amine being substantially in the free state.
7. A method as in claim 6 said alkanol amine having more than one alkyl radical joined to the nitrogen of the amine and each such radical having less than six carbon atoms therein.
8. A method as in claim 6 said alkanol amine being an ethanol amine.
9. A method as in claim 6 said alkanol amine being monoethanol amine.
10. A method for removing grime largely composed of lead sulfide and graphite from brass matrixes for integral line type, said method comprising washing at room temperature the brass matrixes in an aliphatic amine which is liquid at room temperature, and then rinsing the matrix in a chlorinated hydrocarbon liquid having an insoluble acid agent therein without contacting the matrix with the acid agent whereby the chlorinated hydrocarbon absorbs the amine from the

matrix and the amine is subsequently fixed with the acid agent.

11. A method as in claim 10, said agent being an alkali metal bisulfate.

12. A method as in claim 11, said aliphatic amine having less than five carbons in any chain thereof.

13. A method as in claim 12 and said aliphatic amine being an alkanol amine.

14. A method as in claim 13 said alkanol amine being a monoethanol amine. 10

WILLIAM HEINECKE.

#### REFERENCES CITED

The following references are of record in the file of this patent:

#### UNITED STATES PATENTS

| Number    | Name          | Date           |
|-----------|---------------|----------------|
| 1,642,419 | Loew          | Sept. 13, 1927 |
| 1,787,789 | Lovell et al. | Jan. 6, 1931   |
| 1,924,892 | Tuttle        | Aug. 29, 1933  |
| 1,934,076 | Lieber        | Nov. 7, 1933   |
| 2,326,837 | Coleman       | Aug. 17, 1943  |
| 2,418,909 | Skinner       | Apr. 15, 1947  |